

Aug. 31, 1926.

1,598,267

J. A. DE CEW

METHOD OF HYDRATING CELLULOSE FIBERS IN CONCENTRATED STOCK

Filed Feb. 9, 1925



Inventor:

Judson Albert DeCew,  
by Speer, Middleman & Macdonald, Atty.

Patented Aug. 31, 1926.

1,598,267

# UNITED STATES PATENT OFFICE.

JUDSON ALBERT DE CEW, OF MOUNT VERNON, NEW YORK.

## METHOD OF HYDRATING CELLULOSE FIBERS IN CONCENTRATED STOCK.

Application filed February 9, 1925. Serial No. 7,899.

In the manufacture of paper there is a certain class of machinery used for beating or cutting the fibers that is continuous in its operation, pulp and water passing between revolving cones, cylinders or discs, and being rubbed or cut by knives or corrugated surfaces, fastened upon the fixed or moving parts.

Certain types of these machines are called Jordans, Klafins, Marshalls, Bauers, etc., and all operate on similar principles, by passing the fluid pulp between rubbing surfaces.

I have discovered a method of increasing the work done by such machines without increasing the power consumed. The principal method of operating such machines is to allow the liquid pulp to flow into the machine at a concentration of about three parts bone dry fiber to 97 of water, and it is seized by the revolving knives and forced out by centrifugal force into a stock chest.

Under these conditions the space between the knives and the shell is never completely full and the stock being thin and very fluid, a cutting action will take place between the revolving knives as they are brought in contact, which breaks and shortens the fiber.

I have been able to prevent this cutting action and at the same time increase the hydrating action and do more work with the same power by the following methods:—

In the first place I thicken the stock so that the percentage of bone dry fiber is over 4% of the total fluid mass. This partial dehydration may be carried out by allowing the fluid pulp to pass through a revolving wire screen which I call a thickener, such as shown in the figure, which extracts a part of the water so that the pulp fibers come into rubbing contact with each other. Most of the beaters in common use are so constructed that the stock discharged from them is too fluid to give a good jordaning action.

I then allow this stock to flow into the machine through a pipe at a height of ten feet or more above the machine and in order to maintain the pressure from this head I prevent the free discharge of pulp from the outlet of the machine, restricting the opening of the discharge and thus producing a back pressure.

Under these conditions there is an internal pressure of stock within the machine which forces it into all the vacant spaces between the knives and shell by maintaining an in-

ternal pressure of over 5 lbs. per square inch by means of the feed head and restricted discharge and at the same time having more than 4 parts of actual fibers to a 100 of fluid stock. Thus I can obtain surface hydration on the fibers and avoid cutting the fibers when the knives are in contact because the increased number of fibers receiving the blow enables them to resist the pressure without being broken in two.

By this means of operation the fibers will remain longer within the sphere of the rubbing action because they will only be discharged from the machine as the stock is required and the machine will always be operating at high efficiency, whereas at the present time a large proportion of the power used is the friction between the knives which come into contact with other knives of the shell with very little stock between them.

Although the best results are obtained by working on a stock of a concentration of over 4% total solids, nevertheless I can improve the results of any Jordan to a great extent without changing the stock conditions by so restricting the flow of stock from the Jordan that it is backed up all through the Jordan, filling all vacant spaces and also up the feed pipe to a height of 10 feet or over.

The head of the stock at the feeding end, however, is the means used for forcing the stock through the machine at a density of over 4%.

The average Jordan is installed in such a manner that the stock must be thinned to under 4% in order to get the required capacity.

What I claim as my invention is:—

1. A method of hydrating cellulose fibers within a continuous beating machine of the Jordan type with rubbing surfaces, which consists in introducing the stock at a concentration of over 4 parts of stock to 96 parts water and at the same time maintaining a pressure of stock at the inlet to the machine of over 5 pounds per square inch.

2. A method of hydrating cellulose fibers by means of a Jordan engine, which consists in first removing a portion of water from the stock, until it contains more than 4% bone dry fiber, and then forcing this through the Jordan at a pressure greater than 5 pounds per square inch at the Jordan inlet.

3. A method of hydrating cellulose fibers within a continuance beating machine of the

Jordan type, which consists in pumping the pulp stock to a height above the beating machine, then passing it through a thickening device from which it is discharged at a concentration of over 4% total solids into a pipe carrying it to the beating machine, the pipe being filled with stock to a sufficient head to produce a pressure within the machine of over 5 lbs. per square inch.

4. A method of hydrating pulp stock in 10 a Jordan engine, which consists in forcing it through the machine at a concentration of over 4% total solids and at a pressure of over 5 lbs. per square inch at the inlet.

In testimony whereof I affix my signature.

JUDSON ALBERT DE CEW.